# EUROPEAN PATENT SPECIFICATION

(11) **EP 0 934 823 B1**
(45) Date of publication and mention of the grant of the patent: **02.04.2003**
(21) Application number: 99200196.6
(22) Date of filing: 18.01.1999
(51) Int. Cl.: B41C 1/10

(54) **Heat-sensitive imaging material for making lithographic printing plates requiring no processing**
Wärmeempfindliches Aufzeichnungsmaterial und Verfahren zur Herstellung von verarbeitungsfreien Flachdruckformen damit
Elément d'enregistrement de l'image et procédé pour la fabrication de plaques lithographiques sans traitement utilisant cet élément

(30) Priority: 09.02.1998 EP 98200372
(43) Date of publication of application: 11.08.1999
(73) Proprietor: AGFA-GEVAERT, 2640 Mortsel (BE)
(72) Inventor: Vermeersch, Joan, 2640 Mortsel (BE); Van Damme, Marc, 2640 Mortsel (BE); Hauquier, Guy, 2640 Mortsel (BE)

(56) References cited:
- EP-A- 0 573 092
- EP-A- 0 609 941
- EP-A- 0 816 071
- FR-A- 2 240 471

## Description

### FIELD OF THE INVENTION

The present invention relates to a heat-sensitive imaging element for making lithographic printing plates. More specifically the invention relates to a heat-sensitive imaging element which requires no processing.

### BACKGROUND OF THE INVENTION

Lithographic printing is the process of printing from specially prepared surfaces, some areas of which are capable of accepting ink, whereas other areas will not accept ink.

In the art of photolithography, a photographic material is made imagewise receptive to oily or greasy ink in the photo-exposed (negative working) or in the non-exposed areas (positive working) on a ink-repelling background.

In the production of common lithographic plates, also called surface litho plates or planographic printing plates, a support that has affinity to water or obtains such affinity by chemical treatment is coated with a thin layer of a photosensitive composition. Coatings for that purpose include light-sensitive polymer layers containing diazo compounds, dichromate-sensitized hydrophilic colloids and a large variety of synthetic photopolymers. Particularly diazo-sensitized systems are widely used.

Upon imagewise exposure of such light-sensitive layer the exposed image areas become insoluble and the unexposed areas remain soluble. The plate is then developed with a suitable liquid to remove the diazonium salt or diazo resin in the unexposed areas.

On the other hand, methods are known for making printing plates involving the use of imaging elements that are heat-sensitive rather than photosensitive. A particular disadvantage of photosensitive imaging elements such as described above for making a printing plate is that they have to be shielded from the light. Furthermore they have a problem of stability of sensitivity in view of the storage time and they show a lower resolution. The trend towards heat-sensitive printing plate precursors is clearly seen on the market.

**EP-A- 444 786, JP- 63-208036,**and **JP- 63-274592** disclose photopolymer resists that are sensitized to the near IR. So far, none has proved commercially viable and all require wet development to wash off the unexposed regions. **EP-A- 514 145** describes a laser addressed plate in which heat generated by the laser exposure causes particles in the plate coating to melt and coalescence and hence change their solubility characteristics. Once again, wet development is required.
**EP-A- 652 483** discloses a lithographic printing plate requiring no dissolution processing which comprises a substrate bearing a heat-sensitive coating, which coating becomes relatively more hydrophilic under the action of heat. Said system yields a positive working printing plate. **EP-A- 609 941** describes a heat-mode recording material comprising on a substrate a metallic layer and a thin hydrophobic layer which becomes hydrophilic upon exposure. However the lithographic performance of the obtained printing plate is poor.

### OBJECTS OF THE INVENTION

It is an object of the present invention to provide a heat-sensitive imaging element for preparing lithographic printing plates requiring no dissolution processing and having a high lithographic performance (ink acceptance, scratch resistance , durability)

### SUMMARY OF THE INVENTION

According to the present invention there is provided a heat-sensitive imaging element for making lithographc printing plates comprising on a lithographic base, having a hydrophilic surface, a silver layer and on top thereof an oleophilic polymeric layer having a thickness of less than 5 µm characterised in that said polymeric layer comprises a polymer containing phenolic groups.

### DETAILED DESCRIPTION OF THE INVENTION

It has been found that according to the present invention, using an imaging element as described above, lithographic printing plates requiring no processing and having an excellent lithographic performance can be obtained.

The thickness of the silver layer is preferably from 0.01 µm to 2 µm, and most preferably from 0.05 µm to 1.5 µm.

A silver layer for use in this invention as the metallic layer can be made according to the principles of the silver complex diffusion transfer reversal process, hereinafter called DTR-process, having been described e.g. in US-P 2,352,014 and in the book "Photographic Silver Halide Diffusion Processes" by André Rott and Edith Weyde - The Focal Press - London and New York, (1972).

In the DTR-process non-developed silver halide of an information-wise exposed photographic silver halide emulsion layer material is transformed with a so-called silver halide solvent into soluble silver complex compounds which are allowed to diffuse into an image-receiving element and are reduced therein with a developing agent, generally in the presence of physical development nuclei, to form a silver image having reversed image density values (DTR-image) with respect to the black silver image obtained in the exposed areas of the photographic material.

In another method for providing a silver layer on the lithographic base having a hydrophilic surface a silver halide emulsion disposed on a lithographic base having a hydrophilic surface is strongly exposed to actinic radiation and then developed, or otherwise processed to maximum blackness. The black opaque emulsion is converted to a reflective recording material by heating at least to 270 °C in an oxygen containing environment until the emulsion coating assumes a shiny reflective appearance. Such method is disclosed in **US-P-4 314 260.**

According to an alternative method for providing a silver layer on the lithographic base the silver is provided using vapour or vacuum deposition.

In **EP-A-875 889** the vacuum deposition is replaced by coating from an aqueous medium. According to this disclosure a thin metal layer is formed by the following steps :
(1) preparing an aqueous medium containing ions of a metal,
(2) reducing said metal ions by a reducing agent thus forming metal particles,
(3) coating said aqueous medium containing said metal particles on a transparent support.

The oleophilic layer provided on top of the silver layer comprises a polymer containing phenolic groups. Preferred polymers containing phenolic groups are phenolic resins (e.g. novolac) or hydroxyphenyl substituted polymers (e.g. polyhydroxystyrenes). The oleophilic layer has a thickness of less than 5 µm. As a consequence a highly sensitive heat-sensitive imaging element is obtained. The use of a polymer containing phenolic groups furthermore improves the lithographic performance ( ink acceptance, scratch resistance, durability) of the lithographic printing plates obtained according to the present invention.

According to one embodiment of the present invention, the lithographic base having a hydrophilic surface can be an anodised aluminum. A particularly preferred lithographic base having a hydrophilic surface is an electrochemically grained and anodised aluminum support. Most preferably said aluminum support is grained in nitric acid, yielding imaging elements with a higher sensitivity. According to the present invention, an anodised aluminum support may be treated to improve the hydrophilic properties of its surface. For example, the aluminum support may be silicated by treating its surface with a sodium silicate solution at elevated temperature, e.g. 95°C. Alternatively, a phosphate treatment may be applied which involves treating the aluminum oxide surface with a phosphate solution that may further contain an inorganic fluoride. Further, the aluminum oxide surface may be rinsed with a citric acid or citrate solution. This treatment may be carried out at room temperature or can be carried out at a slightly elevated temperature of about 30 to 50°C. A further interesting treatment involves rinsing the aluminum oxide surface with a bicarbonate solution. Still further, the aluminum oxide surface may be treated with polyvinylphosphonic acid, polyvinylmethylphosphonic acid, phosphoric acid esters of polyvinyl alcohol, polyvinylsulphonic acid, polyvinylbenzenesulphonic acid, sulphuric acid esters of polyvinyl alcohol, and acetals of polyvinyl alcohols formed by reaction with a sulphonated aliphatic aldehyde. It is further evident that one or more of these post treatments may be carried out alone or in combination.

According to another embodiment in connection with the present invention, the lithographic base can comprise a flexible support, such as e.g. paper or plastic film, provided with a hardened hydrophilic layer. A particularly suitable hardedned rough hydrophilic layer may be obtained from a hydrophilic binder hardened with a hardening agent such as formaldehyde, glyoxal, polyisocyanate or preferably a hydrolysed tetra-alkylorthosilicate.

As hydrophilic binder there may be used hydrophilic (co)polymers such as for example, homopolymers and copolymers of vinyl alcohol, acrylamide, methylol acrylamide, methylol methacrylamide, acrylic acid, methacrylic acid, hydroxyethyl acrylate, hydroxyethyl methacrylate or maleic anhydride/vinylmethylether copolymers.

A hardened hydrophilic layer on a flexible support used in accordance with the present embodiment preferably also contains substances that increase the mechanical strength and the porosity of the layer e.g. colloidal silica. In addition inert particles of larger size than the colloidal silica can be added e.g. silica prepared according to Stöber as described in J. Colloid and Interface Sci., Vol. 26, 1968, pages 62 to 69 or alumina particles or particles having an average diameter of at least 100 nm which are particles of titanium dioxide or other heavy metal oxides. Incorporation of these particles gives the surface of the hardened hydrophilic layer a uniform rough texture consisting of microscopic hills and valleys.

The thickness of the hardened hydrophilic layer may vary in the range of 0.2 to 25 µm and is preferably 1 to 10 µm.

Particular examples of suitable hardened hydrophilic layers for use in accordance with the present invention are disclosed in **EP-A 601 240, GB-P-1 419 512, FR-P-230 354, US-P-3 971 660, US-P-4 284 705** and **EP-A 514 490.**

As support on which the hydrophilic layer is provided it is particularly preferred to use a plastic film e.g. substrated polyethylene terephthalate film, cellulose acetate film, polystyrene film, polycarbonate film etc... The plastic film support may be opaque or transparent.

It is particularly preferred to use a polyester film support to which an adhesion improving layer has been provided. Particularly suitable adhesion improving layers for use in accordance with the present invention comprise a hydrophilic binder and colloidal silica as disclosed in **EP-A- 619 524, EP-A- 620 502 and EP-A- 619 525.** Preferably, the amount of silica in the adhesion improving layer is between 200 mg per m² and 750 mg per m². Further, the ratio of silica to hydrophilic binder is preferably more than 1 and the surface area of the colloidal silica is preferably at least 300 m² per gram, more preferably a surface area of 500 m² per gram.

In accordance to the method of the present invention for obtaining a lithographic printing plate the heat-sensitive imaging element is image-wise scanning exposed using a laser, preferably a laser that operates in the infrared or near-infrared, i.e. wavelength range of 700-1500nm. Most preferred are laser diodes emitting in the near-infrared.

After the exposure the imaging element can be used without an additional wet treatment as a lithographic printing plate.

The printing plate obtained according to the present invention can also be used in the printing process as a seamless sleeve printing plate. This cylindrical printing plate wich has as diameter the diameter of the print cylinder is slided on the print cylinder instead of applying in a classical way a classically formed printing plate. More details on sleeves are given in 'Grafisch Nieuws' ed. Keesing, 15, 1995, page 4 to 6.

The following examples illustrate the present invention without limiting it thereto. All parts and percentages are by weight unless otherwise specified.

### EXAMPLES

### Example 1 (comparative)

### Preparation of the DTR material

On the back of a polyethylene terephthalate support with a thickness of 175 µm, was coated a layer from a 11% wt solution in demineralized water ( pH=4), with a wet thickness of 50 µm. The resulting layer contained 74.7% of titaniumdioxide, 8.6% of polyvinylalcohol, 16.2% of hydrolysed tetramethylorthosilicate and 0.5% wetting agents.

On the other side of the polyethylene terephthalate support which is provided with a hydrophilic subbing layer, is first coated a layer from a 20% wt solution in demineralized water ( pH=4), with a wet coating thickness of 50 µm. This layer contained 82.7% of titaniumdioxide, 9.1% of polyvinylalcohol, 8.2% of hydrolysed tetramethylorthosilicate and 0.17‰ of palladiumsulphide (particle size 2-3 nm). On this base layer, a layer of palladiumsulphide particles (2-3 nm) is coated from a 0.24‰ wt solution (pH=9) in demineralized water, with a wet thickness of 13 µm. Finally, an emulsion layer and top layer were simultaneously coated by means of the cascade coating technique. The emulsion layer was coated with a wet thickness of 30 µm and such that the silver halide coverage expressed as AgNO₃ was 2.50 g/m² and the gelatin content was 1.50 g/m². The toplayer was coated with a wet thickness of 15 µm such that the gelatin content was 0.7 g/m². The top layer further contained 61 mg/m² of Levanyl Rot and 0.14 g/m² matting agent.

### Preparation of the heat-sensitive imaging element

To obtain a heat-sensitive imaging element according to the present invention, the unexposed DTR material as described above was developed for 12s at 24 °C in an aqueous alkaline solution having the following ingredients:

| | |
|---|---|
| Anhydrous sodium sulphite | 120 g |
| Sodium hydroxide | 22 g |
| Carboxymethylcellulose | 4 g |
| Potassium bromide | 0.75 g |
| Anhydrous sodium thiosulphate | 8 g |
| Aluminum sulphate.18H₂O | 8 g |
| Ethylene diamine tetraacetic acid tetrasodium salt | 4.2 g |
| Hydroquinone | 20 g |
| Methylfenidon | 6.25 g |
| Demineralized water to make pH (25°C) > 12.5 | 1L |

The initiated diffusion transfer was allowed to continue for 18 s to form a silver layer, whereafter the material was rinsed with water containing 0.03‰ of trypsine at 50 °C.

The thus obtained metallic silver layer was provided with a hydrophobic layer by guiding the material through a finisher at 45°C, having the following composition:

| | |
|---|---|
| Dextran 70000 | 40 g |
| Polyethyleneglycol 200 | 50 ml |
| Sodiumdihydrogenphosphate.2H₂O | 20 g |
| Citric acid | 22 g |
| Potassium nitrate | 12.5 g |
| Sodium hydroxide | 12.6 g |
| 1-phenyl-5-mercaptotetrazole | 0.5 g |
| Biocide | 0.1 g |
| Wetting agent | 261.5 mg |
| Demineralized water to make pH (25°C) = 5.95 | 1L |

### Example 2

### Preparation of the DTR material

The DTR material was prepared as described in example 1.

### Preparation of the heat-sensitive imaging element

To obtain a heat-sensitive imaging element according to the present invention, the unexposed DTR material was developed for 12s at 24 °C in an aqueous alkaline solution as described in example 1.

The initiated diffusion transfer was allowed to continue for 18 s to form a silver layer, whereafter the material was rinsed with water at 50 °C.

As comparative examples one of the thus obtained metallic silver layers was used as such, one was coated with a polyethylene layer (2 g/m²) and one was prepared as described in example 1.

As an example of the invention one of the obtained metallic silver layers was coated with a novolac layer (2 g/m² Alnovol SPN452).

### Exposing the heat-sensitive imaging element

The 4 materials were all imaged with a Gerber C42T™ internal drum platesetter at 12,000 rpm (367 m/s, pixel dwell time 0.032 µs) and 2540 dpi. The power level of the laser in the image plane was 5.4 W.

After imaging, the plates were printed without any additional wet treatment.

### Printing the imagewise exposed element

The plates were printed on a Heidelberg GTO46 printing machine under more critical conditions than in example 1 with a conventional ink (K+E) and a fountain solution of 5% G671c (commercialy available from Agfa-Gevaert N.V.) + 10% isopropanol.

The plate that did not get an extra coating layer after developing (comparative example), did not show any ink-uptake in the unexposed areas and the material prepared as described in example 1 (comparative example) showed a slower ink-uptake while the one with polyethylene as a final coating (comparative example), resulted in a better ink-uptake and no scumming, but the image was already damaged after 25 prints. Finally the one with the novolac coating on top (example of the invention), showed a good ink-uptake, no scumming and a runlength > 3000 prints.

### Example 3

### Preparation of the DTR material

The DTR material was prepared as described in example 1 or 2.

### Preparation of the heat-sensitive imaging element

To obtain a heat-sensitive imaging element according to the present invention, the unexposed DTR material was developed for 12s at 24 °C in an aqueous alkaline solution as described in example 1 or 2.

The initiated diffusion tranfer was allowed to continue for 18 s to form a silver layer, whereafter the material was rinsed with water at 50 °C.

As comparative examples one of the thus obtained metallic silver layers was used as such, one was coated with a polyethylene layer (1 g/m²) and one was coated with a top layer of a copolymer of polyvinylbutyral, polyvinylalcohol and polyvinylacetate, esterified with trimellitic acid anhydride (1 g/m²).

As an example of the invention one of the obtained metallic silver layers was coated with a novolac layer (1 g/m² Alnovol SPN452).

### Exposing the heat-sensitive imaging element

The 4 materials were all imaged with a Gerber C42T™ internal drum platesetter at 12,000 rpm (367 m/s, pixel dwell time 0.032 µs) and 2540 dpi. The power level of the laser in the image plane was 5.4 W.

After imaging, the plates were printed without any additional wet treatment.

### Printing the imagewise exposed element

The plates were printed on a Heidelberg GTO46 printing machine with a conventional ink (K+E) and a fountain solution of 5% G671c (commercially available from Agfa-Gevaert N.V.) + 10% isopropanol.

The plate that did not get an extra coating layer after developing (comparative example), did not show any ink-uptake in the unexposed areas. The ones with polyethylene (comparative example) and the one with the copolymer as a final coating (comparative example), resulted in a good ink-uptake and no scumming, but the image was already damaged after 25-50 prints. Finally the one with the novolac coating on top (example of the invention), showed a good ink-uptake, no scumming and a runlength > 3000 prints.

### Example 4

### Preparation of the DTR material

The DTR material was prepared as described in example 1 to 3.

### Preparation of the heat-sensitive imaging element

To obtain a heat-sensitive imaging element according to the present invention, the unexposed DTR material was developed for 12s at 24 °C in an aqueous alkaline solution as described in example 1 to 3.

The initiated diffusion tranfer was allowed to continue for 18 s to form a silver layer, whereafter the material was rinsed with water at 50 °C.

As a comparative example one of the thus obtained metallic silver layers was used as such.

As examples of the invention three other silver layers were coated with a novolac layer of respectively 1, 2 and 5 g/m² Alnovol SPN452.

### Exposing the heat-sensitive imaging element

The 4 materials were all imaged with a Gerber C42T™ internal drum platesetter at 12,000 rpm (367 m/s, pixel dwell time 0.032 µs) and 2540 dpi. The power level of the laser in the image plane was 5.4 W.

After imaging, the plates were cleaned with a dry cotton pad and subsequently printed.

### Printing the imagewise exposed element

The plate that did not get an extra coating layer after developing (comparative example), showed strong ablation during imaging and no residues were left on the exposed parts. The plates with a novolac coating on top of 1 or 2 g/m² Alnovol SPN452, ablated as an easily removable yellow powder, while on the one with a 5 g/m² novolac coating, still ablation residues were found after cleaning (examples of the invention).

The plates were printed on a Heidelberg GTO46 printing machine with a conventional ink (K+E) and a fountain solution of 5% G671c (commercially available from Agfa-Gevaert N.V.) + 10% isopropanol.

The plate that did not get an extra coating layer after developing (comparative example), did not show any ink-uptake in the unexposed areas. All three layers with a novolac coating on top (examples of the invention), showed a good ink-uptake and a runlenght> 3000 prints.

## Claims

1. A heat-sensitive imaging material for making lithographic printing plates comprising on a lithographic base, having a hydrophilic surface, a silver layer and on top thereof an oleophilic polymeric layer having a thickness of less than 5 µm wherein said polymeric layer comprises a polymer containing phenolic groups.

2. A heat-sensitive imaging material according to claim 1 wherein said polymer containing phenolic groups is a phenolic resin or a hydroxyphenyl subsituted polymer.

3. A heat-sensitive imaging material according to any of claims 1 or 2 wherein said silver layer has a thickness between 0.05 and 1.5 µm.

4. A heat-sensitive imaging material according to any of the preceeding claims wherein said lithographic base having a hydrophilic surface is a grained and anodised aluminum support.

5. A heat-sensitive imaging material according to claim 4 wherein the lithographic base having a hydrophilic surface is an anodized aluminum support which has been treated with a compound selected from the group consisting of polyvinylphosphonic acid, polyvinylmethylphosphonic acid, phosphoric acid esters of polyvinyl alcohol, polyvinylsulphonic acid, polyvinylbenzenesulphonic acid, sulphuric acid esters of polyvinyl alcohol, and acetals of polyvinyl alcohols formed by reaction with a sulphonated aliphatic aldehyde.

6. A heat-sensitive imaging material according to any of claims 1 to 3 wherein said lithographic base having a hydrophilic surface comprises a plastic support provided with a hydrophilic binder crosslinked by means of a hydrolysed tetra-alkylorthosilicate.

7. A method for making a lithographic printing plate comprising the step of image-wise exposing to actinic radiation a heat-sensitive element comprising on a lithographic base , having a hydrophilic surface, a metallic layer or metal oxide silver layer and on top thereof an oleophilic polymeric layer having a thickness of less than 5 µm wherein said polymeric layer comprises a polymer containing phenolic groups.

8. A method for making multiple copies of an original comprising the steps of:
- image-wise exposing to actinic radiation a heat-sensitive imaging material comprising on a lithographic base , having a hydrophilic surface, a silver layer and on top thereof an oleophilic polymeric layer having a thickness of less than 5 µm wherein said polymeric layer comprises a polymer containing phenolic groups,
- starting printing without an additional wet treatment of the exposed imaging material.

9. A method according to claim 7 or 8 wherein said image-wise exposure is carried out by an IR-laser.

## Patentansprüche

1. Ein wärmeempfindliches Bilderzeugungsmaterial zur Herstellung von lithografischen Druckplatten, das auf einer lithografischen Unterlage mit einer hydrophilen Oberfläche eine Silberschicht und eine darüber vergossene oleophile polymere Schicht mit einer Stärke von weniger als 5 µm enthält, **dadurch gekennzeichnet, daß** die polymere Schicht ein phenolische Gruppen enthaltendes Polymer enthält.

2. Ein wärmeempfindliches Bilderzeugungsmaterial nach Anspruch 1, **dadurch gekennzeichnet, daß** das phenolische Gruppen enthaltende Polymer ein Phenolharz oder ein hydroxyphenylsubstituiertes Polymer ist.

3. Ein wärmeempfindliches Bilderzeugungsmaterial nach einem der Ansprüche 1 oder 2, **dadurch gekennzeichnet, daß** die Stärke der Silberschicht zwischen 0,05 und 1,5 µm liegt.

4. Ein wärmeempfindliches Bilderzeugungsmaterial nach einem der vorstehenden Ansprüche, **dadurch gekennzeichnet, daß** die lithografische Unterlage mit einer hydrophilen Oberfläche ein gekörnter und eloxierter Aluminiumträger ist.

5. Ein wärmeempfindliches Bilderzeugungsmaterial nach Anspruch 4, **dadurch gekennzeichnet, daß** die lithografische Unterlage mit einer hydrophilen Oberfläche ein eloxierter Aluminiumträger ist, der mit einer Verbindung aus der Gruppe bestehend aus Polyvinylphosphonsäure, Polyvinylmethylphosphonsäure, Phosphorsäureestern von Polyvinylalkohol, Polyvinylsulfonsäure, Polyvinylbenzolsulfonsäure, Schwefelsäureestern von Polyvinylalkohol und Acetalen von Polyvinylalkoholen, die durch Reaktion mit einem sulfonierten alifatischen Aldehyd gebildet sind, verarbeitet ist.

6. Ein wärmeempfindliches Bilderzeugungsmaterial nach einem der Ansprüche 1 bis 3, **dadurch gekennzeichnet, daß** die lithografische Unterlage mit einer hydrophilen Oberfläche einen ein hydrophiles Bindemittel enthaltenden Kunststoffträger enthält, wobei das Bindemittel mittels eines hydrolysierten Tetraalkylorthosilikats vernetzt ist.

7. Ein Verfahren zur Herstellung einer lithografischen Druckplatte, **gekennzeichnet durch** den Schritt, in dem ein wärmeempfindliches Element, das auf einer lithografischen Unterlage mit einer hydrophilen Oberfläche eine Silberschicht und eine darüber vergossene oleophile polymere Schicht mit einer Stärke von weniger als 5 um enthält, bildmäßig mit aktinischer Strahlung belichtet wird, **dadurch gekennzeichnet, daß** die polymere Schicht ein phenolische Gruppen enthaltendes Polymer enthält.

8. Ein durch die nachstehenden Schritte gekennzeichnetes Verfahren zur Herstellung mehrfacher Kopien von einer Vorlage :
- bildmäßige Belichtung mit aktinischer Strahlung von einem wärmeempfindlichen Bilderzeugungsmaterial, das auf einer lithografischen Unterlage mit einer hydrophilen Oberfläche eine Silberschicht und eine darüber vergossene oleophile polymere Schicht mit einer Stärke von weniger als 5 µm enthält, **dadurch gekennzeichnet, daß** die polymere Schicht ein phenolische Gruppen enthaltendes Polymer enthält,
- Beginnen des Druckzyklus ohne zusätzliche Naßverarbeitung des belichteten Bilderzeugungsmaterials.

9. Ein Verfahren nach Anspruch 7 oder 8, **dadurch gekennzeichnet, daß** die bildmäßige Belichtung mit einem IR-Laser durchgeführt wird.

## Revendications

1. Matériau de formation d'image thermosensible pour fabriquer des clichés d'impression lithographique comprenant, sur une base lithographique possédant une surface hydrophile, une couche d'argent et par-dessus cette dernière, une couche polymère oléophile possédant une épaisseur inférieure à 5 µm, dans lequel ladite couche polymère comprend un polymère contenant des groupes phénoliques.

2. Matériau de formation d'image thermosensible selon la revendication 1, dans lequel ledit polymère contenant des groupes phénoliques est une résine phénolique ou un polymère portant un ou plusieurs substituants hydroxyphényle.

3. Matériau de formation d'image thermosensible selon l'une quelconque des revendications 1 et 2, dans lequel ladite couche d'argent possède une épaisseur entre 0,05 et 1,5 µm.

4. Matériau de formation d'image thermosensible selon l'une quelconque des revendications précédentes, dans lequel ladite base lithographique possédant une surface hydrophile est un support en aluminium grainé et anodisé.

5. Matériau de formation d'image thermosensible selon la revendication 4, dans lequel la base lithographique possédant une surface hydrophile est un support d'aluminium anodisé qui a été traité avec un composé choisi parmi le groupe constitué par l'acide polyvinylphosphonique, l'acide polyvinylméthylphosphonique, des esters d'acides phosphoriques d'alcools polyvinyliques, l'acide polyvinylsulfonique, l'acide polyvinylbenzène-sulfonique, des esters d'acides sulfuriques d'alcools polyvinyliques, et des acétals d'alcools polyvinyliques que l'on obtient par réaction avec un aldéhyde aliphatique sulfoné.

6. Matériau de formation d'image thermosensible selon l'une quelconque des revendications 1 à 3, dans lequel ladite base lithographique possédant une surface hydrophile comprend un support en matière plastique muni d'un liant hydrophile réticulé à l'aide d'un orthosilicate de tétraalkyle hydrolysé.

7. Procédé pour fabriquer un cliché d'impression lithographique, comprenant l'étape consistant à exposer en forme d'image, à un rayonnement actinique, un élément thermosensible comprenant, sur une base lithographique possédant les surfaces hydrophiles, une couche d'argent et par-dessus cette dernière une couche polymère oléophile possédant une épaisseur inférieure à 5 µm, dans lequel ladite couche polymère comprend un polymère contenant des groupes phénoliques.

8. Procédé pour faire des copies multiples d'un original, comprenant les étapes consistant à :
- exposer en forme d'image, à un rayonnement actinique, un élément thermosensible comprenant, sur une base lithographique possédant les surfaces hydrophiles, une couche d'argent et par-dessus cette dernière une couche polymère oléophile possédant une épaisseur inférieure à 5 µm, dans lequel ladite couche polymère comprend un polymère contenant des groupes phénoliques,
- démarrer l'impression en l'absence d'un traitement humide supplémentaire du matériau de formation d'image à l'état exposé.

9. Procédé selon la revendication 7 ou 8, dans lequel ladite exposition en forme d'image est mise en oeuvre à l'aide d'un laser infrarouge.
